

April 8, 1924.

1,489,830

S. R. ILLINGWORTH

MANUFACTURE OF ELECTRODES

Filed Oct. 17, 1922



Inventor  
Stewart Roy Illingworth  
by his Attorneys  
Brodman Wright

Patented Apr. 8, 1924.

1,489,830

# UNITED STATES PATENT OFFICE.

STEWART ROY ILLINGWORTH, OF BRYNFEDWEN, RADYR, WALES, ASSIGNOR TO  
ILLINGWORTH CARBONIZATION COMPANY, LIMITED, OF MANCHESTER, ENGLAND.

## MANUFACTURE OF ELECTRODES.

Application filed October 17, 1922. Serial No. 595,111.

To all whom it may concern:

Be it known that I, STEWART ROY ILLINGWORTH, a subject of the King of Great Britain, residing at Brynfedwen, Radyr, Glamorganshire, Wales, have invented new and useful Improvements in the Manufacture of Electrodes, of which the following is a specification.

This invention relates to the manufacture of electrodes, especially those adapted for use in electric furnaces.

In the production of coke from coal two factors have to be considered: (1) the resinic content and (2) the amount of volatile matter evolved at the critical stage of coking just before the mass loses its plasticity. This occurs when the resinic content is not far removed from 5% by weight of the mass.

According to this invention I treat in the manner hereafter described coal containing not less than 5% by weight of resinic matter and in which the volatile matter evolved at the critical stage is low, that is the volatile matter must not exceed 10% and is preferably 7½%. Such coal may be natural coal or coal produced by oxidizing or blending or heating coals.

In the present case the coals to be treated are preferably of a high resinic content that is over 9% and low in ash, say about 5%; phosphorus say .1% and sulphur 1% of the mass after heating to 900° centigrade. But for use in some metallurgical operations the amount of phosphorus should not exceed .05%. In estimating the resinic content no cognizance is taken of resinic substances which decompose below 300° C. Coals suitable as regards the nature of the coal substance can be washed to produce a product of low ash content.

In carrying out this invention the coal as above defined is compressed, heated preferably to a temperature of 600° C. but at least 50° to 100° C. above the temperature of decomposition of resinic matter in the substance, then impregnated with pitch rendered liquid by heat, and carbonised at 800° to 1000° C. or upwards. Preferably the coal is first finely crushed and is preferably kept under compression during the whole of the heating process. The compressed mass may be advantageously perforated with a central hole.

In place of heated pitch a solution of

pitch or a solution of the heavier of the by-products given off during the process may be used.

The annexed drawings show apparatus which may be employed in carrying out the manufacture according to this invention. Figure 1 is a section and Figure 2 a plan of a mould and Figure 3 is a side elevation of the heating and impregnating apparatus. Figure 4 is a diagrammatic view of a complete apparatus for the carrying out of the process disclosed.

*a* is a mould having sides perforated at *b* and a cover *c* perforated at *d*. The mould has in it a plate *e* having a lug *f* and two wedges *g* and *h* by means of which the material is held in the mould.

Referring to Figure 3, *i* is an oven having doors *j* at each end and *k* is a tank having in it a perforated plate *l* pivoted at *m* which plate is raised and lowered by a lifting bar *n*. *o* is a pitch tank connected to the tank *k* by a pipe *p* for supplying the pitch and a return pipe *q* through which pitch is run back into the tank *o*. The tank *k* is connected by a pipe *r* to a pump to evacuate the tank. A rod *s* may be used as indicated in Figures 1 and 2 when it is desired to form a central hole in the electrode.

In carrying out the invention the coal as above defined is stamped into the mould *a* and is held in the same by the plate *e*, lug *f* and wedge *g*. When the mould is charged it is placed in the oven *i* maintained preferably at a temperature of 600° C. but at least 50° to 100° C. above the temperature of decomposition of the resinic matter. When the carbonisation of the charge is complete the mould is withdrawn through the door *j* and the wedge *h* is driven in to hold the mass in place. The cover is then removed from the tank *k* and the perforated plate *l* is raised to such an angle that the mould *a* can be drawn down upon it. The perforated plate *l* is then lowered into the tank *k* and the cover is replaced and the tank *k* is evacuated through the pipe *r*. When the temperature of the tank *k* has cooled to about 250° C. molten pitch from the tank *o* is allowed to enter the tank *k* by the pipe *p* and thence into the mould *a* through the perforations *b* and *d*. The tank *k* is maintained at about 250° C. for half an hour, preferably by means of waste flue gases from the oven *i*, after which the excess

pitch is run back into the tank *o* through the pipe *q*. The mould is then placed in an oven of the same type as the oven *i* and disposed on the opposite side of the tank *k* and is subjected to a heat of 800° to 1000° C. or upwards, after which the mould is passed to a cooling chamber which is evacuated and preferably filled with an inert gas such as cooled flue gases.

- 10 The impregnation with pitch can be repeated in order to get a more homogeneous product and this is particularly advisable in the case of electrodes of a cross section of over 3" square. Also in the case of large 15 electrodes the tank *k* may be advantageously placed under pressure when the electrode is being impregnated.

The ovens are provided with condensing appliances so that the by-products are recovered from which pitch for use in the process may be obtained.

In place of pitch, tar or other bitumen or resinic like product, for example oil pitch, may be used, but I prefer to use a substance 25 which at 900° C. will give a minimum amount of volatile matter and leave a large proportion of its weight as carbon residue without deleterious components such as sulphur.

30 What I claim is:—

1. In the manufacture of electrodes, compressing coal containing not less than 5% by weight of resinic matter and in which the volatile matter evolved at the critical stage 35 is low, heating it to a temperature at least 50° C. above the temperature of decomposition of resinic matter in the coal, impregnating the compressed coal with a carbonaceous substance which at 900° C. gives a 40 minimum amount of volatile matter and leaves a large amount of carbon without deleterious components and then carbonizing.

2. In the manufacture of electrodes, compressing coal containing not less than 5% by weight of resinic matter and in which the volatile matter evolved at the critical stage 45 is low, heating it to a temperature at least 50° C. above the temperature of decomposition of resinic matter in the coal, impregnating the compressed coal with pitch and then carbonizing.

3. In the manufacture of electrodes, compressing coal containing not less than 5% by 55 weight of resinic matter and in which the volatile matter evolved at the critical stage is low, heating it to a temperature at least 50° C. above the temperature of decomposition of resinic matter in the coal, impregnating the compressed coal with pitch rendered liquid by heat and then carbonizing.

4. In the manufacture of electrodes, compressing coal containing not less than 5% by 60 weight of resinic matter and in which the volatile matter evolved at the critical stage

is low, heating it to a temperature of 600° C., impregnating the compressed coal with a carbonaceous substance which at 900° C. gives a minimum amount of volatile matter and leaves a large amount of carbon without 70 deleterious components and then carbonizing.

5. In the manufacture of electrodes, compressing coal containing not less than 5% by weight of resinic matter and in which the volatile matter evolved at the critical stage is low, heating it to a temperature of 600° C., impregnating the compressed coal with pitch and then carbonizing.

6. In the manufacture of electrodes, compressing coal containing not less than 5% by weight of resinic matter and in which the volatile matter evolved at the critical stage is low, heating it to a temperature of 600° C., impregnating the compressed coal 85 with pitch rendered liquid by heat and then carbonizing.

7. In the manufacture of electrodes, finely crushed coal containing not less than 5%, by weight of resinic matter and in which the volatile matter evolved at the critical stage is low, compressing the same about a 90 rod to leave a central perforation in the compressed mass, and heating it whilst under continued compression to a temperature 95 at least 50° C. above the temperature of decomposition of resinic matter in the coal, impregnating the compressed coal with a carbonaceous substance which at 900° C. gives a minimum amount of volatile matter 100 and leaves a large amount of carbon without deleterious components and then carbonizing.

8. In the manufacture of electrodes, finely crushed coal containing not less than 5% by weight of resinic matter and in which the volatile matter evolved at the critical stage is low, compressing the same about a rod to leave a central perforation in the compressed mass, and heating it whilst under continued compression to a temperature at least 50° C. above the temperature of decomposition of resinic matter in the coal, impregnating the compressed coal with pitch and then carbonizing.

9. In the manufacture of electrodes, finely crushing coal containing not less than 5% by weight of resinic matter and in which the volatile matter evolved at the critical stage is low, compressing the same and heating it whilst under continued compression to a 120 temperature at least 50° C. above the temperature of decomposition of resinic matter in the coal, impregnating the compressed coal with a carbonaceous substance which at 900° C. gives a minimum amount of volatile matter and leaves a large amount of carbon without deleterious components and then carbonizing.

10. In the manufacture of electrodes, fine-

ly crushing coal containing not less than 5% by weight of resinic matter and in which the volatile matter evolved at the critical stage is low, compressing the same, and heating it whilst under continued compression to a temperature at least 50° C. above the temperature of decomposition of resinic

matter in the coal, impregnating the compressed coal with pitch and then carbonizing.

In testimony that I claim the foregoing as my invention I have signed my name this 6th day of October, 1922.

STEWART ROY ILLINGWORTH.